

# UNITED STATES PATENT OFFICE.

WILLIAM E. SAWYER, OF NEW YORK, AND ALBON MAN, OF BROOKLYN,  
N. Y., ASSIGNEES TO ELECTRO DYNAMIC LIGHT COMPANY.

## CARBON FOR ELECTRIC LIGHTS.

SPECIFICATION forming part of Letters Patent No. 229,335, dated June 29, 1880

Application filed November 22, 1878.

*To all whom it may concern:*

Be it known that we, WILLIAM EDWARD SAWYER, of the city, county, and State of New York, and ALBON MAN, of Brooklyn, county 5 of Kings, and State aforesaid, have jointly invented certain Improvements in Carbons for Electric Lights; and we do hereby declare the following to be a description of the same, and of the manner and process of making, constructing, and using them, in such full, clear, concise, and exact terms as will enable any person skilled in the art or science to which it appertains, or with which it is most nearly connected, to make, construct, and use the 15 same, reference being had to certain Letters Patent of the United States heretofore granted to us for certain inventions hereunto appertaining, and to which especial reference will hereinafter be made.

Our invention consists of a new article of manufacture, consisting of an improved illuminating conductor for electric lamps, composed of consolidated carbon created by electric action.

In Letters Patent of the United States No. 205,144, granted to us, we have shown and described an electric lamp, in which a pencil of carbon is heated to incandescence in a nitrogen or other carbon-preservative atmosphere.

One of the principal obstacles to successful electric lighting by incandescence is the dissociated character of nearly all obtainable carbon. In most of such carbon there is danger of fracture as well as of the establishment of 35 the voltaic arc; and, furthermore, the carbon, unless specially prepared by our process, naturally occludes sufficient air or oxygen to render its consumption a mere question of time, since, as fully set forth in the Letters Patent referred to, the least quantity of oxygen in a sealed lamp is sufficient to combust an indefinite quantity of carbon.

As is well known, carbon suitable for electric lighting by the voltaic arc is naturally produced in gas-retorts; but generally the rods or carbons used in the "regulator-lamps," so-called, are molded from the powdered material. Neither the one nor the other quality of carbon is suitable for electric lighting by incandescence. In both there is a lack of homo-

geneity. The pencil is not sufficiently hard and dense, because, in the first place, the heat required to produce the proper character of carbon is as high as 7,000° Fahrenheit, and such a temperature is not obtainable in the retort; and in the second place the mechanical subdivisions of the material and the pressure necessary to produce the perfect article are practically unattainable. Carbon of the ordinary sort, when heated by the electric current, exhibits points and lines of unequal brilliancy. Carbon prepared by our process, when so heated, glows with a uniform brilliancy throughout.

We have found that a pencil of carbon immersed in a hydrocarbon gas or liquid and heated to an extremely high temperature by the voltaic current is not itself attacked, but decomposes the surrounding matter, the carbon of which enters and fills up its pores to an extent impossible except with matter in a very attenuated state, and deposits a perfectly homogeneous layer, generally of a bright gray color, upon the exterior surface. As the carbon increases in size more current is required to maintain its temperature, and if the current is gradually increased in accordance with the demand for it there is apparently no limit to the increase in mass of the homogeneous exterior deposit. Carbon pencils may be cut from this deposit, or the original pencil with its coating may be used in the lamps.

In this process it would seem that the carbon is never in contact with the liquid in which it is immersed, but surrounded by a carbon gas of a very high temperature. Naphtha, turpentine, beeswax, balsam, and most oils, if pure, operate satisfactorily. Almost any hydrocarbon, in fact, will answer.

We do not confine ourselves to the treatment of carbon alone, since it is obvious that many infusible substances, non-conductors of electricity, may be heated in hydrocarbon liquids or gases, so as to render them conductors of electricity—as, for instance, a tube of lime inclosing a pencil of carbon, through which the electric current is caused to circulate.

In the Letters Patent hereinbefore referred to we have described a method of charging a

55

60

65

70

75

80

85

90

95

100

sealed globe with pure nitrogen gas. We will suppose that the pencil of carbon, held between two carbon pieces of greater mass than that of the pencil, as shown in the said Letters Patent, is immersed in the hydrocarbon liquid and heated in the manner already described. Being then cleansed in alcohol, the pencil and its holders, without having been disturbed, are placed in the globe, in which they are to be hermetically sealed. The globe is charged with pure nitrogen, and then, while still allowing pure nitrogen to flow into and out of the globe, we heat the carbon to incandescence, thus driving out all impurities and 15 occluded gases, which are carried out of the lamp by the current of nitrogen.

With this operation the preparation of the carbon is completed, and the lamp, now being hermetically sealed, as described in the Letters Patent referred to, is ready for use.

Having thus described our invention, we claim and desire to secure by Letters Patent—

Carbon consolidated and purified by electrically treating it, in combination with a carbonaceous substance, for the production of electric burners.

WILLIAM EDWARD SAWYER.  
ALBON MAN.

Witnesses:

AMOS BROADNAX,  
THOS. CROCKER.